

## UNITED STATES PATENT OFFICE.

LESTER KIRSCHBRAUN, OF CHICAGO, ILLINOIS.

## WATERPROOFING MATERIAL AND PROCESS OF MAKING THE SAME.

No Drawing. Application filed April 14, 1921, Serial No. 461,377. Renewed October 28, 1926.

This invention relates to improvements in waterproofing material and a process of making the same and refers more particularly to a method of combining a bituminous binder with pulp or fibrous material to form a waterproofing substance.

Among the salient objects of the invention are to provide a process incorporating comminuted particles of a bituminous binder 10 with a fibrous stock, the binder being incorporated into the body of the stock in a finely divided form and while in a relatively non-adhesive state; to provide a process in which a finely comminuted binder substance, such 15 as bituminous materials, asphalt or the like, in discrete form, is treated and mixed with a pulp or paper stock and the mixture run over a machine for forming it into sheets of various thicknesses; to provide a process in 20 which the relatively small particles of the binder are provided with an enveloping agent and are subsequently mixed with the fibrous stock from which sheets are formed on a paper or other sheet-forming machine and 25 finally the sheets subjected to heat whereby the fusible binder is caused to melt and agglomerate about the fibrous stock, and to provide a process in which the enveloping agent carries and precipitates the binder upon 30 the fibres attaching it more fixedly thereto.

Heretofore, sheets have been made in which a comminuted asphaltic or bituminous substance has been mixed with the pulp or fibrous stock and run over a sheet-forming machine 35 or molded. Such processes have been more or less successful where the binder used has been pitch so hard as to possess the properties of an inert filler rather than a binder with adhesive properties at normal temperatures. 40 Among such pitches may be mentioned gilsonite, grahamite, hard coal-tar pitch, rosin and even harder pitch of petroleum distillation which can be readily ground or reduced by mechanical means to a comminuted form. 45 Where, however, the pitches are of such character as to possess any appreciable adhesive-ness, such as is characteristic of the softer varieties of pitch, the introduction of such material into the paper stock has not re-sulted in a successful operation, owing to the tendency to gum the blankets, wires, driers and other essential parts of the ma-chine.

While the softer and more adhesive bitu-minous binder may be rendered non-adhesive and most advantageously operable on a paper

machine by emulsification rather than by the herein disclosed process, nevertheless, binders, which are somewhat adhesive at normal temperatures, may be successfully 60 introduced and handled on a paper machine by the present invention.

As distinguished from the binders usable in the present process the harder pitches are of such a refractory nature as to be incapable 65 of spreading through the sheet, but remain in comminuted form in the finished product, requiring immersion in a hot waterproofing substance or solvent to melt the particles and produce a body sufficiently continuous to 70 achieve a waterproof product.

It will be understood, of course, that even the refractory pitches will be more effectively precipitated on to the fibres and carried into the sheet.

The process disclosed in the present invention consists briefly, first, in mixing asphaltic, bituminous or other fusible waterproof binder materials ground or reduced to a finely divided condition or in comminuted 80 form in water with an agent which has the properties of causing coagulation or precipi-tation of the binder particles on the fibres or forming upon the particles of binder en-veloping coatings. Various agents may be 85 used to produce this enveloping coating about the binder substance, preferably silicate of soda precipitated with aluminum sulphate, tri-sodium phosphate and zinc sulphate, tan-ning liquors and sulphite liquors precipitated 90 with aluminum sulphate or analogous pre-cipitates may be employed. The disclosure is not limited to the use of these agents, but includes such treatment as will produce, when observed microscopically, a nucleus of com-95 minuted pitch surrounded by a protective medium or a distinct tendency of the binder particles to be precipitated upon the fibres. The coating is produced by the action of the above-named agents added to the aqueous 100 binder suspension in their proper order.

The present invention does not contem-plate the emulsification of binder substances such as disclosed in United States Letters Patent 1,302,810, issued May 6th, 1919, in 105 which asphalt is very finely dispersed in emulsified form, but has to do with the en-veloping of binder particles reduced mechani-cally to comminuted form and subsequently treated in the manner described. The com-minuted asphalt so treated may be mixed 110 with a fibrous stock and run over a paper

machine or other forming mechanisms and subsequently dried during which the enveloping medium is broken so that the binder attaches itself to the fibres and incorporates therewith to produce a waterproof sheet.

I claim as my invention:

1. A process of making a waterproof-composition-containing material, comprising reducing bituminous waterproofing material to relatively dry comminuted form, enveloping the waterproofing material with a protective coating, mixing said material with fibrous stock and felting the stock to form a sheet.

2. A process of making a waterproof composition-containing material, comprising reducing bituminous waterproofing material to relatively dry comminuted form, subsequently enveloping the waterproofing material with a protective coating, mixing said material with fibrous stock and felting the stock to form a sheet.

3. A process of making a waterproof-composition-containing material, comprising reducing bituminous waterproofing material to comminuted form, enveloping the waterproofing material with a protective coating, precipitating the waterproofing material on fibrous stock and forming the stock into sheets.

4. A process of making waterproof composition, comprising reducing a waterproof binder to comminuted form, coating the binder with a protective film, precipitating the binder on fibrous stock, forming the stock into sheets, and breaking the protective film.

5. A process of making waterproof composition, comprising reducing a waterproof binder to comminuted form, coating the binder with a protective film, precipitating the binder on fibrous stock, forming the stock into sheets, and breaking the protective film by the removal of water and the action of heat.

6. Waterproof composition comprising a felted fibrous sheet and a comminuted waterproof bituminous binder precipitated on the fibres.

7. A process of making a waterproof-composition-containing material, comprising re-

ducing bituminous waterproofing material to comminuted form, and enveloping the waterproofing material with a protective substance.

8. A process of making a waterproof-composition-containing material, comprising reducing normally adhesive bituminous waterproofing material to comminuted form, and enveloping the waterproofing material with a protective coating, thereby rendering the composition non-adhesive.

9. A waterproof-composition-containing material, comprising a base of comminuted bituminous substance, rendered non-adhesive by the addition thereto of an enveloping agent, said bituminous substance having the characteristics of having been comminuted by mechanical action.

10. A process of making a waterproof-composition-containing material comprising enveloping pitchy waterproofing material in finely divided comminuted condition with a protective coating, precipitating the waterproofing material on fibrous stock and forming the stock into sheets.

11. A composition capable of being sheeted comprising a fibrous stock and a comminuted waterproofing bituminous binder precipitated on the fibres.

12. A process of making a waterproof-composition-containing material comprising reducing a bitumen-pitch type waterproofing material to comminuted form by mechanical action, and enveloping the waterproofing material with a protective substance.

13. A process of making a waterproof-composition-containing material comprising comminuting a bitumen-pitch type waterproofing material and enveloping same with a protective coating.

14. A waterproof composition-containing material comprising finely divided bitumen-pitch type waterproofing material as a binder rendered non-adhesive by the addition thereto of an enveloping agent, said binder having the characteristics of having been finely divided by mechanical action, and fibre added to the mixture.

LESTER KIRSCHBRAUN.